

## UNITED STATES PATENT OFFICE

2,186,733

## COLOR PHOTOGRAPHY

Wilhelm Schneider and Alfred Fröhlich, Dessau, Germany, assignors, by means assignments, to Agfa Ansco Corporation, Binghamton, N. Y., a corporation of Delaware

No Drawing. Application September 18, 1937, Serial No. 164,499. In Germany October 7, 1936

13 Claims. (Cl. 95—6)

Our present invention relates to color photography and more particularly to improved color components for the process of color development.

It has for an object to provide color components which are soluble in water and which are fast to diffusion with respect to the silver halide emulsion.

A further object of the invention is to provide a new and improved process for preparing color formers having these properties.

A further object is to provide silver halide emulsions containing the color components fast to diffusion.

A further object is to provide an improved film for color photography having superposed silver halide emulsion layers, each layer containing a color component fast to diffusion.

A known process for producing color photographic and cinematographic pictures uses silver halide emulsion layers which contain color formers. The production of the picture varies with the kind of color former used. As described in U. S. Patents 1,102,028 and 1,055,155 there may be used color formers which yield color pictures during the development with certain developing substances. For producing multi-color pictures it has been proposed to superimpose light-sensitive layers containing various coupling bodies, the layers being separated from each other by intermediate layers so that diffusion of the coupling bodies from the light-sensitive layers may be prevented. It has been found, however, that this expedient for preventing diffusion is not sufficiently successful in practice. In U. S. Patents 2,179,228, 2,178,612, and 2,179,244 and U. S. patent applications Ser. No. 94,340 filed August 5, 1936, and Ser. No. 159,518, filed August 17, 1937, there are described dyestuff components which are fast to diffusion.

The present invention is based on the observation that color formers of good fastness to diffusion are obtainable by the introduction into the molecule of the dyestuff component as a substituent, a constituent or a conversion product of a natural resin. The conversion products, however, are limited to those in which the general structure of the natural resin is substantially retained. The constituent or conversion product of the natural resin must contain a reactive group, for instance a carboxyl group or a hydroxyl group, with the aid of which the color former can be caused to enter into chemical combination. Suitable resinous products are, for example,  $\alpha$ -pimarabietic acid,  $\beta$ -pimarabietic acid, pinabietic acid, abietic acid, dihydropinabietic acid, siaresinolic acid, sumaresinolic acid,  $\alpha$ -amyrin and various resinoles and bitter substances, for example the humulone of hops.

The compounds of the resinous product with

the dyestuff former may be made in any known manner, either by producing an ester-like or acid amide-like union between the hydroxy- or the amino-group of the dyestuff former and the acid group of the resin acid or by producing an ether-like union, for instance between the hydroxy-group of the resinole and the hydroxy-group of the dyestuff former. For further guidance to those skilled in the art reference is here made to the examples, which disclose in detail the actual process to be followed. They do not, however, limit the invention to the specific data disclosed there, but all such equivalent processes are within the ambit of the invention as fall within the scope of the annexed claims.

As dyestuff components into which the residue of the resin product is to be introduced there may be named, for example, aminonaphthols, aminonaphthol-carboxylic acids or sulfonic acids, aminophenols, aminophenylmethylpyrazolone, hydroxyphenylmethylpyrazolones, aminobenzoyl-acetic acid ester arylides, aminonaphthoyl-acetic acid ester arylides, acylacetic acid ester amino-arylides and substitution products of these bodies.

When the dyestuff component of this kind, that is to say containing a resin constitution, is added to a photographic silver halide emulsion the color picture may be produced, according to the nature of the dyestuff component, by color development or through the intermediary of diazo-compounds or by the silver bleaching-out process. The procedure may be that described in any of the following: U. S. Patent 2,179,228 and U. S. patent application Ser. No. 141,093, filed May 6, 1937, and in any of the U. S. patents or U. S. patent applications enumerated on page 1, column 1, lines 35 to 38. Or the components located in multi-layer film may be converted into azo-dyes following development and fixing by treatment with a diazo compound such as a carbonic acid solution of tetrazotized benzidine disulfonic acid. There is thus produced in each emulsion layer together with a silver picture a dyestuff in which no structure can be perceived by magnification. The film is then treated with a silver bleaching out bath, i. e. that described in British Patent 401,340 to produce the dye image.

The dyestuff formers used in the foregoing process are, in consequence of the groups in the dyestuff molecules which lend solubility in water, of themselves or in the form of their salts soluble in water and may therefore be incorporated without difficulty in the photographic silver halide emulsion at any point in the process of the production. The resinous substituent makes the dyestuff component fast to diffusion. It must be observed, however, that the chlorides of the resin acids must be used as homogeneous compounds. The silver halide emulsions made in accordance

with the invention are applied in known manner for making photographic layers, which may be on one or both faces of a carrier and may be sensitized for different regions of the spectrum. If 5 desired the silver halide emulsion layers may be combined with the other emulsion layers in which color pictures may be produced by any other process, for example by mordant dyeing or toning.

The emulsions may be prepared in any other 10 manner, for example differently sensitized emulsions having different dyestuff formers may be brought in the form of small particles on the surface of the carrier.

The following examples illustrate the invention:

(1) 30 grams of the purest colophony are converted in known manner into abietic acid chloride and the benzene solution of this is added in drops to a solution of 18 grams of 1-amino-5-naphthol in 100 cc. of pyridine so that by application of external heat the benzene dropped in is continuously distilled off. When all the amino-naphthol has entered into reaction with the abietic chloride the product is precipitated by 25 means of ice and after the mass has been rendered acid to Congo by hydrochloric acid it is filtered and the solid matter washed. The latter is the dyestuff component which is to be added to the silver halide emulsion.

(2) 25 grams of 3'-amino-5'-sulfo-1-phenyl-3-methyl-5-pyrazolone are dissolved in 100 cc. of pyridine. Into the solution there is dropped a solution of 30 grams of abietic acid chloride in benzene, the addition being so made that the 35 benzene is continuously distilled off. When all the aminosulfonylpyrazolone has entered into reaction the whole is precipitated by means of ice, then made acid to Congo by means of hydrochloric acid and filtered, the solid matter 40 being washed neutral with water.

20 grams of the dyestuff component thus obtained are added to 1 kilo of emulsion and the latter is then poured to form a layer. After exposure the layer is developed with a solution 45 alkaline with sodium carbonate of aminodimethylaniline, whereby there is obtained a red color image in addition to the silver image. The latter is removed in known manner, whereby the red color image remains.

50 If the exposed silver halide emulsion layer is developed not with aminodimethylaniline but with an ordinary black-and-white developer and the silver image is converted into a silver anti-diazotate of  $\beta$ -naphthyl-amine, for example as 55 described in U. S. patent application Ser. No. 10,704, filed March 12, 1935, and finally this anti-diazotate silver image is treated with a weak acid solution, a yellow picture is obtained.

Instead of converting the silver image into the 60 diazo-image there may be produced throughout the whole layer a uniform red dyestuff by treating the layer with a solution of tetrazotized benzidine disulfonic acid and destroying the red dyestuff at the places of the silver image by the 65 silver bleaching-out process with use of known agents.

(3) A three-layer film for three-color photography is made in the following manner. 70 1 kilo of silver bromide emulsion is mixed with 15 grams of para-abietylaminobenzoylacetate acid anilide-para-carboxylic acid. In the layer of this emulsion there may be produced by means of color development a yellow dyestuff image. Also dyestuff images which may be produced with 75 aid of diazo-compounds are yellow.

For making the second emulsion layer 1 kilo of silver bromide emulsion is mixed with a sensitizer for green and then with 15 grams of a solution of 3-abietylamino-5-sulfo-1-phenyl-3-methyl-5-pyrazolone. In this layer there is produced by color development a purple dyestuff image.

For making the third emulsion layer 1 kilo of silver bromide emulsion is mixed with a sensitizer for red and with a solution of 15 grams of 1-abietylamino-5-hydroxynaphthalene-8-carboxylic acid. In this layer chromogenic development produces a blue-green dyestuff image.

If desired the several layers of emulsion may be alternated with filter layers.

What we claim is:

1. A photographic silver halide emulsion for color photography comprising abietyl-amino-naphthol.

2. A photographic silver halide emulsion for color photography comprising 3-abietyl-amino-5-sulfo-1-phenyl-3-methyl-5-pyrazolone.

3. A silver halide emulsion for color photography containing a color former having a natural resin linked thereto by a homopolar linkage.

4. A silver halide emulsion for color photography containing a color former having a natural resin linked thereto by a homopolar linkage, said natural resin being a member of the group consisting of pimarabietic acid, pinabietic acid, 30 abietic acid, stearinolic- and sumaresinolic acids, amyrins, resinoles and humulones.

5. A silver halide emulsion for color photography containing a natural resin-acid-amide of a color former.

6. A process which comprises developing with an aromatic amino developer a silver halide emulsion for color photography containing a color former having a natural resin linked thereto by homopolar linkages.

7. A process which comprises developing with an aromatic amino developer, a silver halide emulsion for color photography containing a color former having a natural resin linked thereto by homopolar linkage, said natural resin being a member of the group consisting of pimarabietic acid, pinabietic acid, abietic acid, stearinolic- and sumaresinolic acids, amyrins, resinoles and humulones.

8. A process which comprises developing with an aromatic amino developer, a silver halide emulsion for color photography containing a natural resin-acid amide of a color former.

9. The silver halide emulsion defined in claim 3 wherein the homopolar linkage is selected from the class consisting of an ether-, an ester-, and an acid amide linkage.

10. The silver halide emulsion defined in claim 5 wherein the resin acid is abietic acid.

11. The silver halide emulsion defined in claim 5 wherein the color former is a pyrazolone and the resin acid is abietic acid.

12. A photographic silver halide gelatine emulsion for color photography comprising abietyl-aminosulfonylpyrazolone.

13. A silver halide emulsion for color photography containing a color former having linked thereto by a homopolar linkage a resinous substance selected from the class consisting of a natural resin and its derivatives in which the molecular structure of said natural resin is substantially retained.

WILHELM SCHNEIDER.  
ALFRED FRÖHLICH.